

## 1

2,946,676

## FERROCHROMIUM-ALUMINUM ALLOY

Joseph H. Brennan, Niagara Falls, and Earle R. Saunders, Grand Island, N.Y., assignors to Union Carbide Corporation, a corporation of New York

No Drawing. Continuation of application Ser. No. 421,182, Apr. 5, 1954. This application Apr. 29, 1957, Ser. No. 655,500

7 Claims. (Cl. 75—27)

This invention relates to an improved ferroalloy, and more particularly concerns an improved ferrochromium-aluminum alloy, which may be used as an alloy addition for an exothermic reaction mixture.

The current popular practice of employing alloy addition agents in exothermic reaction mixtures for the production of ferrous alloys has created a need for new and improved alloy additions. In order for an alloy to be suitable for use in an exothermic reaction mixture, it must be capable of acting as a reducing agent in the exothermic reaction and as an alloy addition for a ferrous melt. It must be non-reactive at ambient temperatures with the oxidant of the exothermic mixture. It should be capable of reacting exothermically when added to the melt to produce a sufficient quantity of heat to reduce substantially the temperature drop normally accompanying such addition. It must not only be suitable for use as an addition agent in melts requiring the propagation of heat, but as an effective non-exothermic alloy addition as well.

Aluminum possesses all of the above attributes which are desirable in an alloy addition to be added to a ferrous melt. Specifically, aluminum reacts exothermically with certain oxidizing agents like sodium nitrate or sodium bichromate to generate an extremely large amount of heat. With the aid of the heat released by the exothermic reaction, it is possible to add proportionately large quantities of alloying material to a steel bath without producing any objectionable temperature drop in the bath.

It is, therefore, an object of the present invention to provide a new and improved aluminum-bearing ferroalloy that is suited for use as an alloy addition to a ferrous melt.

Another object of the invention is to provide a novel aluminum-bearing ferroalloy which is suitable for use as a reducing agent in an exothermic reaction mixture.

Yet another object of the present invention is to provide a ferrous alloy containing aluminum and chromium in such correlated proportions that the alloy is suitable for use in either aluminum-bearing products or as a reducing agent in an exothermic reaction mixture.

The objects of the invention are achieved by forming an aluminum-bearing ferroalloy containing essentially chromium and iron constituents for alloying in a ferrous bath. Preferably, the alloy of the invention comprises aluminum, chromium, iron, optional amounts of silicon and carbon, and the usual impurities. In a preferred embodiment of the invention, the range of composition of the alloy should be within the following limits.

|          | Percent   |
|----------|-----------|
| Aluminum | 5 to 85   |
| Chromium | 5 to 70   |
| Iron     | 1.5 to 36 |
| Silicon  | Up to 30  |
| Carbon   | Up to 5   |

Small amounts of other elements may be introduced or may enter as incidental impurities.

## 2

Within the above range the ratio of chromium to iron should be between 1.5 to 1 and 4 to 1.

According to the present invention, ferrochromium-aluminum alloys within the above composition range are useful as alloy additions for the production of aluminum-bearing steels, and preferably as reducing agents in exothermic mixtures.

When used as a reducing agent, the aluminum content of the instant alloy is very powerfully exothermic in reaction with such commonly used oxidants as sodium nitrate or sodium bichromate. However, it is to be pointed out that alloys of the above specified range of composition are not necessarily restricted to oxidation of the aluminum when other possible reducing agents, like silicon and carbon are also present. For example, in exothermic mixtures employing sodium nitrate as an oxidant, successful restriction of the aluminum oxidation depends upon the presence of a minimum of a stoichiometric quantity of aluminum for reaction with all of the sodium nitrate. Otherwise the sodium nitrate preferentially reacts with the aluminum, silicon and carbon contents in the alloy in the order named until all of the sodium nitrate is exhausted. Such a reaction has much less efficiency because the heat producing capacities of silicon and carbon are approximately one-half to one-fourth that produced by the reaction of aluminum with sodium nitrate. For this reason an excess of aluminum is usually preferred in reactions with sodium nitrate.

The specific example next to be referred to is illustrative of the selective type of exothermic reaction obtained when a ferrochromium-aluminum alloy of the present invention is employed as a reducing agent in an exothermic reaction mixture.

In a one-ton arc furnace heat, briquettes having a composition of 0.54% carbon, 4.97% aluminum, 24.60% silicon and 8.0% sodium nitrate were added to a steel melt. Before the briquettes were added, the steel melt contained 0.07% carbon, 0.04% silicon, 0.01% aluminum, remainder iron. After adding the above briquettes, the composition of the steel melt was 0.09% carbon, 1.10% silicon and 0.02% aluminum, indicating a 100% carbon recovery from the briquettes, an 83% recovery of silicon and a 4% aluminum recovery.

It is desirable that the ferrochromium-aluminum alloy embodied in the present invention be easily reduced to powder form for obvious metallurgical reasons. Although the instant alloy composition possesses favorable pulverulent properties, it is also susceptible of reduction to a fine particle size by a novel yet effective method.

50 This method consists in alloying aluminum with high carbon ferrochromium to produce an alloy in which much of the carbon is present as aluminum carbide, and leaching the resulting alloy with water. The aluminum carbide of the alloy reacts with the water to form hydrocarbon gas and aluminum hydrate. This reaction causes the alloy to crumble and reduces it to a fine powder and at the same time substantially lowers the carbon content of the alloy.

55 The effectiveness of this method of decarburization depends, of course, on the proportion of carbon present in the subject alloy as aluminum carbide. Investigation has shown that beginning at about 25% aluminum content, increasing proportions of the carbon present in the alloy are in the form of aluminum carbide. At aluminum levels of 50% and over, practically all of the carbon in the alloy is present as aluminum carbide.

However, for reducing the alloy to a satisfactorily fine powder form, the alloy must have at least 50% aluminum. Best results are obtained when the aluminum content of the instant ferrochromium-aluminum alloy is between 50% and 65% by weight.

The following example illustrates the decarbonization

effect of water on a typical ferrochromium-aluminum alloy embodying the principles of the present invention. Before subjecting the alloy to a leaching operation it comprised 29.90% chromium, 54.79% aluminum, 2.20% carbon, 1.01% silicon and the remainder substantially all iron. After water leaching the carbon content amounted to 0.06%, indicating a percentage loss of carbon of 97%.

From the above it will be evident that the composition of the alloy of the present invention may be varied over a considerably wide range. Generally, however, the particular application that is contemplated or the specific end product desired determines the composition range of the alloy. Listed below in Table I are preferred composition ranges of ferro-chromium-aluminum alloys for use in exothermic mixes, which include alloys having either low carbon content, high carbon content, or high silicon content. The composition of these alloys lie in the broad range envisioned by this invention, but apply to a limited portion thereof.

Table I

|         | High Carbon Alloy, percent | Low Carbon Alloy, percent | High Silicon Alloy, percent |
|---------|----------------------------|---------------------------|-----------------------------|
| Al..... | 5 to 25                    | 45 to 75                  | 5 to 25                     |
| Cr..... | 45 to 70                   | 15 to 40                  | 35 to 55                    |
| Fe..... | 15 to 30                   | 5 to 20                   | 10 to 25                    |
| Si..... | Up to 10                   | Up to 10                  | Up to 30                    |
| C.....  | 0.2 to 5                   | Up to 0.2                 | Up to 2                     |

It will be noted from the above table that in the low carbon alloy the aluminum content is greater than in the high carbon alloy. A higher aluminum content is necessary to allow it to combine with the carbon in the form of aluminum carbide, and thus permit removal of the latter by the previously disclosed water leaching operation.

It is to be understood that modifications and variations may be effected without departing from the novel concepts of the present invention.

This application is a continuation of application Serial No. 421,182, filed April 5, 1954, now abandoned.

What is claimed is:

1. In the manufacture of an alloy steel employing an exothermic reaction mixture as an additive material the improvement which comprises incorporating in said mixture an alloy having aluminum as an exothermic reducing agent therein, the alloy comprising from 5% to 85% aluminum, 5% to 70% chromium, silicon in an amount up to 30%, carbon in an amount up to 5% and the remainder iron, the ratio of said chromium to said iron being at least 1.5 to 1 and not more than 4 to 1.

2. In the manufacture of an alloy steel employing an exothermic reaction mixture as an additive material the improvement which comprises incorporating in said mixture an alloy having aluminum as an exothermic reducing agent therein, the alloy comprising from 45% to 75% aluminum, 15% to 40% chromium, silicon in an amount up to 10%, carbon in an amount up to 2%, and the remainder iron.

3. In the manufacture of an alloy steel employing an exothermic reaction mixture as an additive material the improvement which comprises incorporating in said mixture an alloy having aluminum as an exothermic reducing agent therein, the alloy comprising from 5% to 25% aluminum, 35% to 55% chromium, silicon in an amount up to 30%, carbon in an amount up to 2%, and the remainder iron.

4. In the manufacture of an alloy steel employing an exothermic reaction mixture as an additive material the improvement which comprises incorporating in said mixture an alloy having aluminum as an exothermic reducing agent therein, the alloy comprising from 5% to 25% aluminum, 45% to 70% chromium, silicon in an amount up to 30%, carbon from 0.2% to 5%, and the remainder iron.

5. A low carbon ferrochromium-aluminum alloy for admixture with an oxygen-containing oxidizing agent to provide an exothermic alloy addition mixture and being characterized by the property of self-disintegration upon the addition of water, said alloy containing aluminum between 45% and 75%, chromium between 15% and 40%, silicon up to 10%, carbon between 0.2% and 2%, and the remainder iron and incidental impurities.

6. A ferrochromium-aluminum alloy for admixture with an oxygen-containing oxidizing agent to provide an exothermic alloy addition mixture comprising aluminum between 5% and 25%, chromium between 35% and 55%, silicon up to 30%, carbon up to 2% and the remainder iron and incidental impurities, the ratio of said chromium to said iron being between 1.5 to 1.0 and 4.0 to 1.0.

7. A high carbon ferrochromium-aluminum alloy for admixture with an oxygen-containing oxidizing agent to provide an exothermic alloy addition mixture comprising aluminum between 5% and 25%, chromium between 45% and 70%, silicon up to 10%, carbon between 0.2% and 5% and the remainder iron and incidental impurities.

#### References Cited in the file of this patent

#### UNITED STATES PATENTS

|           |         |               |
|-----------|---------|---------------|
| 1,421,471 | Heskett | July 4, 1922  |
| 2,367,630 | Udy     | Jan. 16, 1945 |
| 2,836,486 | Brennan | May 27, 1958  |

#### OTHER REFERENCES

Kornilov: "Iron Alloys," vol. I, Iron-Chromium-Aluminum Alloys, 1945, 192 pages (in Russian); published by the Academy of Science, Moscow, U.S.S.R.

The Journal of the Iron and Steel Institute, No. 1, 1914, pages 731-733; published by the Iron and Steel Institute, London, England.

The Foundry Trade Journal, vol. 36, July-Sept. 1927, pages 170-171; published by the Institute of British Foundrymen, London, England.

"Aluminum in Iron and Steel," 1953, pages 289 and 448; published by John Wiley and Sons, New York, N.Y., edited by Case and Van Horn. (Publication based upon report by Kornilov in 1945.)